

Patented Sept. 29, 1925.

## UNITED STATES PATENT OFFICE.

WILHELM ROHN, OF HANAU, GERMANY.

PROCESS FOR MAKING PARTS FOR THE MANUFACTURE OF HIGH-VACUUM TUBES AND  
THE LIKE.

No Drawing.

Application filed May 14, 1920. Serial No. 381,519.

*To all whom it may concern:*

Be it known that I, WILHELM ROHN, a citizen of Germany, and resident of Hanau, Germany, have invented new and useful Processes for Making Parts for the Manufacture of High-Vacuum Tubes and the like (for which I have filed application in Germany April 18, 1918), of which the following is a specification.

- 10 It is known that in making high vacuum tubes, such as Röntgen tubes, incandescent cathode tubes, amplifier and valve tubes, tubes for wireless telegraphy and the like particular difficulties are encountered in rendering the metals contained in such tubes free from gases. Attempts have been made to remove the gases from these metals, while evacuating the tubes, by heating them to an excessive degree either directly from outside, or by highly overcharging the tubes. It was, however, found impossible to fully free the metals from gases, even by a protracted treatment, as every fresh rise of temperature causes gas to emerge afresh from the metals, which then rendered the tubes useless. On the other hand an overheating of the parts contained in the tube frequently resulted in turning into dust the metals or the like.
- 20 30 The inventor has described his British Patent No. 138,648, dated May 19, 1921, a process invented by himself, by which a sufficient degasification of metals and alloys of metals is obtained by the said metals and alloys of metals being kept molten for some time under a constant, but very low pressure, or being remelted several times under the

said conditions. Suitable metals and alloys for this treatment are: magnesium, aluminum, copper, silver, gold, nickel, iron, chromium, platinum, alloys of nickel and iron with manganese, silicon, cobalt, chromium, molybdenum, tungsten, as well as alloys of nickel with iron and copper. The 40 preferential metals and alloys for use in 45 vacuum tubes are: aluminum, copper, nickel, iron, and alloys of nickel with iron, copper, chromium or manganese, as well as of iron with manganese and chromium.

In doing so it has been found that such 50 metals or the like, when rolled into sheets or drawn into wire, or when annealed in the presence of any gases, such as hydrogen, will no more absorb noxious quantities of gases 55 and will therefore give no cause for trouble in making the hereinbefore mentioned tubes.

What I claim is:

1. The process of preparing inner metallic parts for use in high vacuum tubes and the like comprising repeatedly heating the desired metal to a molten condition under a constant but very low pressure, and thereafter, annealing the said metal.

2. The process of preparing inner metallic parts for high vacuum tubes and the like comprising repeatedly heating the desired metal to a molten condition under a constant but very low pressure and thereafter mechanically forming said metal into desired shape.

In testimony, that I claim the foregoing as my invention I have signed my name this 27 day of February 1920.

DR. WILHELM ROHN.